

# UNITED STATES PATENT OFFICE.

CARL J. JOHNSON, OF LOUISVILLE, KENTUCKY.

## PROCESS OF TREATING TRANSMISSION-BANDS.

1,293,107.

Specification of Letters Patent.

Patented Feb. 4, 1913.

No Drawing.

Application filed June 1, 1913. Serial No. 237,627.

To all whom it may concern:

Be it known that I, CARL J. JOHNSON, a citizen of the United States, residing at Louisville, in the county of Jefferson and State of Kentucky, have invented certain new and useful Improvements in Processes of Treating Transmission-Bands, of which the following is a specification.

This invention has for its object the treatment of fabric bands, employed as transmission, brake, and clutch bands, and particularly those employed on planetary transmission gears in automobiles, trucks, etc., in such manner that their durability and efficiency will be increased and the "chattering" now frequently noticeable will be eliminated.

In the practice of my improved process, I employ a mixture of powdered or flake graphite, paraffin, and hard grease, such as is commonly known as cup grease, in the proportions, by volume, of fifty per cent. graphite, forty-five per cent. paraffin, and five per cent. grease. The paraffin and grease are heated until liquid and the graphite is then added and the mixture stirred until it is a homogeneous mass. The strap or band to be treated is boiled in this mixture until it is completely impregnated and is then removed and permitted to cool whereupon it will be ready for use.

During the boiling of the band, the paraffin and grease will penetrate the fabric and graphite will be thereby carried into the body of the fabric as well as deposited on the surface thereof.

Straps, bands, and the like treated according to my process remain pliable under all conditions and their surfaces do not become glazed or hardened by reason of their contact with the brake or gear drum and the "chattering", which is caused by the sudden gripping and releasing of the brake or transmission drum, is eliminated and a smooth even friction obtained. The "chattering" is very annoying to the operator and is also destructive of the band and of the mechanism. Bands or straps treated according to my process are, therefore, more durable and efficient than bands not so treated.

Having thus described my invention, what is claimed as new is:

1. A fabric strap impregnated with paraffin, grease, and graphite.
2. The process of treating fabric straps which consists in boiling the same in a mixture containing fifty per cent. of graphite, forty-five per cent. of paraffin, and five per cent. of grease.

In testimony whereof I affix my signature.

CARL J. JOHNSON. [L.S.]